



US006326339B1

(12) **United States Patent**  
**Rattinger et al.**

(10) **Patent No.:** **US 6,326,339 B1**  
(b4) **Date of Patent:** **\*Dec. 4, 2001**

(54) **CLEANSING SYSTEM COMPRISING  
SYNTHETIC DETERGENT BAR AND POUF**

(75) Inventors: **Gail Beth Rattinger**, Teaneck, NJ (US); **Peter Boettcher**, Sterling Forest, NY (US); **Laurie Ann Coyle**, Park Ridge; **William Narath**, Parsippany, both of NJ (US)

(73) Assignee: **Lever Brothers Company, division of Conopco, Inc.**, New York, NY (US)

(\*) Notice: This patent issued on a continued prosecution application filed under 37 CFR 1.53(d), and is subject to the twenty year patent term provisions of 35 U.S.C. 154(a)(2).

Subject to any disclaimer, the term of this patent is extended or adjusted under 35 U.S.C. 154(b) by 0 days.

This patent is subject to a terminal disclaimer.

(21) Appl. No.: **09/033,008**

(22) Filed: **Mar. 2, 1998**

**Related U.S. Application Data**

(60) Provisional application No. 60/039,501, filed on Mar. 4, 1997.

(51) **Int. Cl.** <sup>7</sup> **C11D 17/04; A47K 7/02**

(52) **U.S. Cl.** **510/140; 510/141; 510/142; 510/439; 510/447; 401/201**

(58) **Field of Search** **510/140, 141, 510/142, 439, 447; 401/201**

(56) **References Cited**

**U.S. PATENT DOCUMENTS**

|           |        |          |           |
|-----------|--------|----------|-----------|
| 1,292,982 | 1/1919 | Wolf     | 401/266   |
| 1,905,163 | 4/1933 | Farquhar | 401/291   |
| 2,079,600 | 5/1937 | Brooks   | 15/104.93 |

|           |          |                  |           |
|-----------|----------|------------------|-----------|
| 2,621,355 | 12/1952  | Fisher           | 15/104.93 |
| 2,817,865 | 12/1957  | Arioli           | 401/201   |
| 2,958,885 | 11/1960  | Donney           | 401/196   |
| 3,167,805 | 2/1965   | Zuppinger et al. | 15/568    |
| 3,175,331 | 3/1965   | Klein            | 401/201   |
| 3,206,152 | 9/1965   | Wimmer           | 401/8     |
| 3,283,357 | 11/1966  | Decker et al.    | 15/104.93 |
| 3,689,437 | * 9/1972 | McLaughlin       | 510/158   |
| 4,151,105 | * 4/1979 | O'Roark          | 510/151   |
| 4,154,542 | * 5/1979 | Rasmason         | 401/7     |
| 4,190,550 | 2/1980   | Campbell         | 401/201   |
| 4,211,675 | * 7/1980 | Machin           | 510/151   |
| 4,228,834 | 10/1980  | Desnick          | 383/13    |
| 4,254,530 | * 3/1981 | Lambert          | 15/235    |
| 4,480,939 | 11/1984  | Upton            | 401/201   |
| 4,574,053 | * 3/1986 | Kinsman et al.   | 510/141   |

(List continued on next page.)

**FOREIGN PATENT DOCUMENTS**

|          |           |       |
|----------|-----------|-------|
| 1220069  | * 1/1971  | (EP). |
| 9207931  | * 5/1992  | (WO). |
| 9216610  | * 10/1992 | (WO). |
| 95/00116 | 1/1995    | (WO). |
| 9526710  | * 10/1995 | (WO). |

**OTHER PUBLICATIONS**

Label—Jean Nate ® “Moisturizing Body Wash Seascape”, undated.

Neutrogena Rainbath Shower Care Line—Three New Products (4 pp.), 1992.

Primary Examiner—Lorna M. Douyon

(74) Attorney, Agent, or Firm—Ronald A. Koatz

(57) **ABSTRACT**

A cleansing system comprises a synthetic detergent bar and a pouf/sponge for holding the bar. By using pouf, it has been found that lather can be enhanced, even in compositions comprising lather depressing emollients. The system also helps decrease perception of mush. A preferred emollient of the invention comprises emollient/oil.

**6 Claims, 2 Drawing Sheets**



## U.S. PATENT DOCUMENTS

|           |         |                  |                         |           |           |         |                          |                       |         |
|-----------|---------|------------------|-------------------------|-----------|-----------|---------|--------------------------|-----------------------|---------|
| 4,613,446 | 9/1986  | Magyar .....     | 15/104.93               | 5,372,751 | *         | 12/1994 | Rys-Cicciari et al. .... | 510/130               |         |
| 4,792,443 | *       | 12/1988          | Filomeno .....          | 424/62    | 5,462,378 | 10/1995 | Webb .....               | 401/201               |         |
| 4,969,225 | *       | 11/1990          | Schubert .....          | 15/209 C  | 5,520,840 | *       | 5/1996                   | Massaro et al. ....   | 510/151 |
| 5,022,517 | 6/1991  | Benitez .....    | 206/77.1                | 5,723,432 | *         | 3/1998  | Beerse et al. ....       | 510/447               |         |
| 5,031,759 | 7/1991  | Ogilvie .....    | 206/77.1                | 5,756,438 | *         | 5/1998  | Rau et al. ....          | 510/151               |         |
| 5,144,744 | 9/1992  | Campagnoli ..... | 29/446                  | 5,916,856 | *         | 6/1999  | Massaro et al. ....      | 510/141               |         |
| 5,284,598 | *       | 2/1994           | Subramanyam et al. .... | 510/153   | 6,042,288 | *       | 3/2000                   | Rattinger et al. .... | 401/201 |
| 5,300,249 | *       | 4/1994           | Schwartz et al. ....    | 510/153   | 6,114,291 | *       | 9/2000                   | He et al. ....        | 510/152 |
| 5,366,125 | 11/1994 | Procido .....    | 224/622                 |           |           |         |                          |                       |         |

\* cited by examiner

**FIG. 1**  
(PRIOR ART)



**FIG. 2**  
(PRIOR ART)



**FIG. 3**  
(PRIOR ART)



*FIG. 4*



## CLEANSING SYSTEM COMPRISING SYNTHETIC DETERGENT BAR AND POUF

This application claims the benefit of Provisional Application No. 60/039,501, filed Mar. 4, 1997.

5

### FIELD OF THE INVENTION

The present invention relates to personal cleansing systems or kits comprising synthetic detergent bars and a personal cleansing hand held bath sponge, particularly one containing moisturizing components.

### BACKGROUND OF THE INVENTION

U.S. Pat. No. 5,144,744 to Campagnali et al. teaches the type of polymeric meshed sponge contemplated by this invention. There is no teaching, however, of its use with bar soaps.

WO 95/00116 (assigned to Procter & Gamble) teaches the use of these polymeric sponges in a system comprising liquid cleanser and moisturizer.

These references do not teach or recognize the use of polymeric meshed sponge with synthetic surfactant bars, for example, bars containing 5-90%, preferably 10-80% surfactant. Use of the sponges can remedy some of the deficiencies found in synthetic bars and not found in pure soap bars. For example, a synthetic bar, particular one comprising lesser amounts of surfactants and more structurant (e.g., 5-60% surfactant, preferably 10-50% surfactant and 10-40% structurant such as polyalkylene glycol) may be a less moisturizing bar and therefore require benefit agents/moisturizers. Often these oily moisturizing agents are lather depressants. Use of the bar pouf retainer allows these relatively low surfactant, moisturizer-containing bars to be utilized without sacrificing lather. In addition, synthetic bars tend to be softer/mushier than pure soap bars. Use of the bar polymeric meshed sponge provides sensory signals which allow the consumer to sense less mush. Lesser lather and mush perception are not problems normally associated with non-synthetic soap bar.

In about 1993, Neutrogena introduced a Rainbar® product which was advertised with a body polishing sponge. It is believed, however, that the Neutrogena bar did not comprise 10% to 80% (by weight of bar) acyl isethionate, let alone the preferred isethionate and zwitterionic surfactant system of the invention. Bynum Concepts® also had a sponge product (Bodykiss®) advertised to use with bar soap. Again, there is no teaching or suggestion to use with synthetic surfactants, let alone specifically acyl isethionate.

Finally, preferred tubular mesh holders provide other advantages one would expect from a nylon mesh bag such as stimulating skin with the rough material; and/or allowing bars to be readily held during the lathering experience.

### BRIEF SUMMARY OF THE INVENTION

The present invention relates to a soap bar cleansing system comprising:

- (1) a synthetic surfactant bar composition comprising:
  - (a) 5% to 90% by wt., preferably 20% to 60% by wt. synthetic surfactant selected from the group consisting of anionic, nonionic, amphoteric, cationic surfactants and mixtures thereof and wherein the surfactant system comprises at least 10%, preferably 15-80% by wt. total bar of acyl isethionate, i.e., C<sub>8</sub>-C<sub>24</sub>, preferably C<sub>8</sub>-C<sub>18</sub> acyl isethionate; and
  - (b) 10% to 90% by wt., preferably 20% to 60% by wt. of a bar structurant selected from the group consist-

ing of C<sub>8</sub> to C<sub>24</sub> fatty acids, ester derivatives; C<sub>8</sub> to C<sub>24</sub> alcohols or ether derivatives thereof; polyalkylene glycols having MW between 1000 and 100,000, water soluble starches (e.g., maltodextrin); and hydrophobically modified water soluble polymers (e.g., EO-PO block copolymers or hydrophobically modified PEG); and

- (2) a light weight polymeric meshed personal cleansing hand held sponge; wherein said sponge is in a form suitable for use as a hand held cleansing implement.

The surfactant bar composition of the invention may comprise 5% to 60% surfactant and greater amounts of structurant relative to surfactant. In addition, it may comprise benefit agent.

In one embodiment the composition comprises:

- (a) 5 to 60% surfactant (comprising at least 10%, by wt. of bar, acyl isethionate);
- (b) 10% to 70% by wt. structurant; and
- (c) 0.01 to 15% benefit agent/emollient.

### DESCRIPTION OF THE FIGURES

FIGS. 1-3 are picture of polymeric meshed material as a sponge (no insert) of prior art.

Specifically:

FIG. 1 is a perspective representation of a diamond mesh polymeric sponge. Rope handle 7 may be used for the pouf.

FIG. 2 is a picture showing how the sponge can be held in the hand.

FIG. 3 shows netting mesh which can be used to make the sponge.

The ease with which a cleaning polymeric mesh sponge can be held in the hand for cleaning is shown in FIG. 2. A security band 13 holds the multi-layered netting mesh together to form the polymeric mesh sponge.

The netting mesh that can be used in making the polymeric mesh sponge is illustrated in FIG. 3 wherein 21 represents the mesh in stretched position. The fine polymeric filaments used in making the netting are represented by 18 with 19 representing the spot bonding of the filaments to form the open mesh 20.

FIG. 4 is a figure of a particular pouf "bag" designed to hold a bar inserted therein. The figure shows bag in closed position (bar would be inside) with drawstring pulled to close bag. The bag is made of polymeric meshed material.

### DETAILED DESCRIPTION OF INVENTION

The present invention relates to a cleansing system comprising a bar composition and a sponge/pouf completely.

More specifically, the system comprises:

- (1) a synthetic surfactant bar composition comprising:
  - (a) 5% to 90% by wt., preferably 20% to 60% by wt. synthetic surfactant selected from the group consisting of anionic, nonionic, amphoteric and cationic surfactants and mixtures thereof; and
  - (b) 10% to 90% preferably 20 to 60% by wt. of a bar structurant and/or filler selected from the group consisting of C<sub>8</sub> to C<sub>24</sub> fatty acid or ester derivatives thereof or salts of fatty acid thereof; C<sub>8</sub> to C<sub>24</sub> alcohols or ether derivatives thereof; polyalkylene glycol having MW between 1000 and 100,000, preferably 200 and 20,000, starches and hydrophobically modified water soluble polymers such as EO-PO block copolymers or hydrophobically modified polyalkylene glycol; and

(2) a light weight polymeric meshed personal cleansing hand held sponge;  
wherein said sponge is in a form suitable for use in a hand held cleansing implement.

## Bar Composition

## Surfactant System

The anionic detergent active which may be used may be aliphatic sulfonates, such as a primary alkane (e.g., C<sub>8</sub>–C<sub>22</sub>) sulfonate, primary alkane (e.g., C<sub>8</sub>–C<sub>22</sub>) disulfonate, C<sub>8</sub>–C<sub>22</sub> alkene sulfonate, C<sub>8</sub>–C<sub>22</sub> hydroxyalkane sulfonate or alkyl glyceryl ether sulfonate (AGS); or aromatic sulfonates such as alkyl benzene sulfonate.

The anionic may also be an alkyl sulfate (e.g., C<sub>12</sub>–C<sub>18</sub> alkyl sulfate) or alkyl ether sulfate (including alkyl glyceryl ether sulfates). Among the alkyl ether sulfates are those having the formula:



wherein R is an alkyl or alkenyl having 8 to 18 carbons, preferably 12 to 18 carbons, n has an average value of greater than 1.0, preferably greater than 3; and M is a solubilizing cation such as sodium, potassium, ammonium or substituted ammonium. Ammonium and sodium lauryl ether sulfates are preferred.

The anionic may also be alkyl sulfosuccinates (including mono- and dialkyl, e.g., C<sub>6</sub>–C<sub>22</sub> sulfosuccinates); alkyl and acyl taurates, alkyl and acyl sarcosinates, sulfoacetates, C<sub>8</sub>–C<sub>22</sub> alkyl phosphates and phosphates, alkyl phosphate esters and alkoxy alkyl phosphate esters, acyl lactates, C<sub>8</sub>–C<sub>22</sub> monoalkyl succinates and maleates, sulfoacetates, alkyl glucosides and acyl isethionates. Sulfosuccinates may be monoalkyl sulfosuccinates having the formula:



and

amide-MEA sulfosuccinates of the formula;



wherein R<sup>4</sup> ranges from C<sub>8</sub>–C<sub>22</sub> alkyl and M is a solubilizing cation.

Sarcosinates are generally indicated by the formula:



wherein R<sup>1</sup> ranges from C<sub>8</sub>–C<sub>20</sub> alkyl and M is a solubilizing cation.

Taurates are generally identified by formula:



wherein R<sup>2</sup> ranges from C<sub>8</sub>–C<sub>20</sub> alkyl, R<sup>3</sup> ranges from C<sub>1</sub>–C<sub>4</sub> alkyl and M is a solubilizing cation.

Particularly preferred are the C<sub>8</sub>–C<sub>18</sub> acyl isethionates. These esters are prepared by reaction between alkali metal isethionate with mixed aliphatic fatty acids having from 6 to 18 carbon atoms and an iodine value of less than 20. At least 75% of the mixed fatty acids have from 12 to 18 carbon atoms and up to 25% have from 6 to 10 carbon atoms.

Acyl isethionates, when present, will generally range from about 10% to about 70% by weight of the total bar composition. Preferably, this component is present from about 30% to about 60%.

The acyl isethionate may be an alkoxyolated isethionate such as is described in llardi et al., U.S. Pat. No. 5,393,466, hereby incorporated by reference. This compound has the general formula:



wherein R is an alkyl group having 8 to 18 carbons, m is an integer from 1 to 4, X and Y are hydrogen or an alkyl group having 1 to 4 carbons and M<sup>+</sup> is a monovalent cation such as, for example, sodium, potassium or ammonium.

It should be understood that the bar may comprise a certain amount of soap as anionic surfactant. Since the invention is related to use of synthetic surfactants inside a sponge, however, it will be understood that there must be a minimum level of synthetic, i.e., at least 5% of all surfactant, preferably at least 20%, more preferably, at least 50% of all surfactant and most preferably 60 to 100% of the surfactant system.

When used, the term "soap" is used in its popular sense, i.e., alkali metal or alkanol ammonium salt of aliphatic alkane or alkene monocarboxylic acids. Sodium, potassium, mono-, di- and triethanol ammonium cations, or combinations thereof, are suitable for purposes of the invention.

Generally, sodium soaps are used. Soaps useful herein are the well known alkali metal salts of natural or synthetic aliphatic (alkanoic or alkenoic) acids having 13 to 22 carbons, preferably 12 to 18. They may be described as alkali metal carboxylates of acrylic hydrocarbons having about 12 to 22 carbons.

Amphoteric surfactants which may be used in this invention include at least one acid group. This may be a carboxylic or a sulphonate acid group. They include quaternary nitrogen and therefore are quaternary amido acids. They should generally include an alkyl or alkenyl group of 7 to 18 carbon atoms. They will usually comply with an overall structural formula:



where R<sup>1</sup> is alkyl or alkenyl of 7 to 18 carbon atoms;

R<sup>2</sup> and R<sup>3</sup> are each independently alkyl, hydroxyalkyl or carboxyalkyl of 1 to 3 carbon atoms;

m is 2 to 4;

n is 0 to 1;

X is alkylene of 1 to 3 carbon atoms optionally substituted with hydroxyl, and Y is —CO<sub>2</sub>— or —SO<sub>3</sub>—

Suitable amphoteric surfactants within the above general formula include simple betaines of formula:



and amido betaines of formula:



where  $n$  is 2 or 3.

In both formulae  $\text{R}^1$ ,  $\text{R}^2$  and  $\text{R}^3$  are as defined previously.  $\text{R}^1$  may in particular be a mixture of  $\text{C}_{12}$  and  $\text{C}_{14}$  alkyl groups derived from coconut so that at least half, preferably at least three quarters of the groups  $\text{R}^1$  have 10 to 14 carbon atoms.  $\text{R}^2$  and  $\text{R}^3$  are preferably methyl.

A further possibility is that the amphoteric detergent is a sulphobetaine of formula:



or



where  $m$  is 2 or 3, or variants of these in which  $-(\text{CH}_2)_3\text{SO}_3^-$  is replaced by



In these formulae  $\text{R}^1$ ,  $\text{R}^2$  and  $\text{R}^3$  are as discussed previously.

The nonionics which may be used include in particular the reaction products of compounds having a hydrophobic group and a reactive hydrogen atom, for example aliphatic alcohols, acids, amides or alkylphenols with alkylene oxides, especially ethylene oxide either alone or with propylene oxide. Specific nonionic detergent compounds are alkyl ( $\text{C}_6$ – $\text{C}_{22}$ ) phenols ethylene oxide condensates, the condensation products of aliphatic ( $\text{C}_8$ – $\text{C}_{18}$ ) primary or secondary linear or branched alcohols with ethylene oxide, and products made by condensation of ethylene oxide with the reaction products of propylene oxide and ethylenediamine. Other so-called nonionic detergent compounds include long chain tertiary amine oxides, long chain tertiary phosphine oxides and dialkyl sulphoxides.

The nonionic may also be a sugar amide, such as a polysaccharide amide. Specifically, the surfactant may be one of the lactobionamides described in U.S. Pat. No. 5,389,279 to Au et al. which is hereby incorporated by reference or it may be one of the sugar amides described in U.S. Pat. No. 5,009,814 to Kelkenberg, hereby incorporated into the subject application by reference.

Examples of cationic detergents are the quaternary ammonium compounds such as alkyltrimethylammonium halogenides.

Other surfactants which may be used are described in U.S. Pat. No. 3,723,325 to Parran Jr. and "Surface Active Agents and Detergents" (Vol. I & II) by Schwartz, Perry & Berch, both of which are also incorporated into the subject application by reference.

One preferable surfactant system comprises:

- 10 (a) a first synthetic surfactant which is anionic; and  
 (b) a second synthetic surfactant selected from the group consisting of a second anionic different from the first, a nonionic, an amphoteric and mixtures thereof.

The first anionic can be any of those recited above, but is 15 preferably a  $\text{C}_8$  to  $\text{C}_{18}$  isethionate as discussed above. Preferably acyl isethionate will comprise 10% to 90% by wt. total bar composition.

The second surfactant is preferably a sulfosuccinate, a betaine or mixtures of the two. The second surfactant or mixture of surfactant will generally comprise 1% to 10% total bar composition. A particularly preferred composition comprises enough sulfosuccinate to form 3–8% total bar compositions and enough betaine to form 1–5% of total bar composition.

#### Structuring Aids and/or Fillers

20 25 The compositions may also contain 10 to 90% by wt., preferably 20 to 80% by wt. of a structurant and/or filler. Such structurants can be used to enhance the bar integrity, improve the processing properties, and enhance desired user sensory profiles.

30 The structurant is generally long chain, preferably straight and saturated, ( $\text{C}_8$ – $\text{C}_{24}$ ) fatty acid or ester derivative thereof; and/or branched long chain, preferably straight and saturated, ( $\text{C}_8$ – $\text{C}_{24}$ ) alcohol or ether derivatives thereof.

A preferred bar structurant is polyalkylene glycol with 35 molecular weight between 2000 and 20,000, preferably between 3000 and 10,000. Those PEGs are commercially available, such as those marketed under the tradename of CARBOWAX SENTRY PEG8000® or PEG4000® by Union Carbide.

Other ingredients that can be used as structurants or fillers 40 include starches, preferably water soluble starches such as maltodextrin and polyethylene wax or paraffin wax.

Structuring aids can also be selected from water soluble polymers chemically modified with hydrophobic moiety or moieties, for example, EO-PO block copolymer, hydrophobically modified PEGs such as POE(200)-glyceryl-stearate, glucam DOE 120 (PEG 120 Methyl Glucose Dioleate), and Hodag CSA-102 (PEG-150 stearate), and Rewoderm® (PEG modified glyceryl cocoate, palmitate or tallowate) from Rewo Chemicals.

50 Other structuring aids which may be used include Amerchol Polymer HM 1500 (Nonoxynol Hydroethyl Cellulose). Optional Ingredients

In addition, the bar compositions of the invention may include 0 to 15% by wt. optional ingredients as follows:

55 perfumes; sequestering agents, such as tetrasodium ethylenediaminetetraacetate (EDTA), EHDP or mixtures in an amount of 0.01 to 1%, preferably 0.01 to 0.05%; and coloring agents, opacifiers and pearlizers such as zinc stearate, magnesium stearate,  $\text{TiO}_2$ , EGMS (ethylene glycol monostearate) or Lytron 621 (Styrene/Acrylate copolymer); 60 all of which are useful in enhancing the appearance or cosmetic properties of the product.

The compositions may further comprise antimicrobials such as 2-hydroxy-4,2'4' trichlorodiphenylether (DP300); preservatives such as dimethyloldimethylhydantoin (Glydant XL1000), parabens, sorbic acid etc.

The compositions may also comprise coconut acyl mono- or diethanol amides as suds boosters, and strongly ionizing

salts such as sodium chloride and sodium sulfate may also be used to advantage.

Antioxidants such as, for example, butylated hydroxytoluene (BHT) may be used advantageously in amounts of about 0.01% or higher if appropriate.

Cationic polymers as conditioners which may be used include Quatrisoft LM-200 Polyquaternium-24, Merquat Plus 3330 ·Polyquaternium 39; and Jaguar® type conditioners.

Polyethylene glycols as conditioners which may be used include:

|        |           |             |
|--------|-----------|-------------|
| Polyox | WSR-205   | PEG 14M,    |
| Polyox | WSR-N-60K | PEG 45M, or |
| Polyox | WSR-N-750 | PEG 7M.     |

Another ingredient which may be included are exfoliants such as polyoxyethylene beads, walnut shells and apricot seeds.

Water

Compositions of the invention also comprise 1% to 10% by wt., preferably 4% to 7% by wt. water.

In one embodiment of the invention, the bar composition comprises no more than about 70% surfactant. Said compositions also contain 10% to 70% by wt. structurant/filler.

Because of lower surfactant levels, such compositions would be more "drying" on the skin and such compositions would comprise 0.01 to 10% benefit agent/emollient.

A preferred composition comprises:

- (1) 10% to 60% by wt. surfactant as defined above;
- (2) 10% to 35% by wt. structurant/filler as defined above; and
- (3) 0.01 to 10% emollient/benefit agent.

The benefit agent "composition" may be a single benefit agent component or it may be a benefit agent compound added via a carrier. Further the benefit agent composition may be a mixture of two or more compounds one or all of which may have a beneficial aspect. In addition, the benefit agent itself may act as a carrier for other components one may wish to add to the bar composition.

The benefit agent can be an "emollient oil" by which is meant a substance which softens the skin (stratum corneum) by increasing into water content and keeping it soft by retarding decrease of water content.

Preferred emollients include:

- (a) silicone oils, gums and modifications thereof such as linear and cyclic polydimethylsiloxanes; amino, alkyl alkylaryl and aryl silicone oils;
- (b) fats and oils including natural fats and oils such as jojoba, soybean, rice bran, avocado, almond, olive, sesame, persic, castor, coconut, mink oils; cacao fat; beef tallow, lard; hardened oils obtained by hydrogenating the aforementioned oils; and synthetic mono, di and triglycerides such as myristic acid glyceride and 2-ethylhexanoic acid glyceride;
- (c) waxes such as carnauba, spermaceti, beeswax, lanolin and derivatives thereof;
- (d) hydrophobic plant extracts;
- (e) hydrocarbons such as liquid paraffins, vaseline, micro-crystalline wax, ceresin, squalene, pristan and mineral oil;
- (f) higher fatty acids such as lauric, myristic, palmitic, stearic, behenic, oleic, linoleic, linolenic, lanolic, isostearic and poly unsaturated fatty acids (PUFA);
- (g) higher alcohols such as lauryl, cetyl, stearyl, oleyl, behenyl, cholesterol and 2-hexydecanol alcohol;

(h) esters such as cetyl octanoate, myristyl lactate, cetyl lactate, isopropyl myristate, myristyl myristate, isopropyl palmitate, isopropyl adipate, butyl stearate, decyl oleate, cholesterol isostearate, glycerol monostearate, glycerol distearate, glycerol tristearate, alkyl lactate, alkyl citrate and alkyl tartrate;

(i) essential oils such as mentha, jasmine, camphor, white cedar, bitter orange peel, rya, turpentine, cinnamon, bergamot, citrus unshiu, calamus, pine, lavender, bay, clove, hiba, eucalyptus, lemon, starflower, thyme, peppermint, rose, sage, menthol, cineole, eugenol, citral, citronelle, borneol, linalool, geraniol, evening primrose, camphor, thymol, spirantol, penene, limonene and terpenoid oils;

(j) lipids such as cholesterol, ceramides, sucrose esters and pseudo-ceramides as described in European Patent Specification No. 556,957;

(k) vitamins such as vitamin A and E, and vitamin alkyl esters, including those vitamin C alkyl esters;

(l) sunscreens such as octyl methoxyl cinnamate (Parsol MCX) and butyl methoxy benzoylmethane (Parsol 1789);

(m) phospholipids; and

(n) mixtures of any of the foregoing components.

A particularly preferred benefit agent is silicone, preferably silicones having viscosity greater than about 10,000 centipoise. The silicone may be a gum and/or it may be a mixture of silicones. One example is polydimethylsiloxane having viscosity of about 60,000 centistokes.

## II Sponge/Implement

The cleansing system of the invention additionally comprises a light weight polymeric meshed personal hand held sponge.

The cleansing polymeric mesh sponge can be prepared from readily available raw materials or with specially designed mesh materials. The polymeric mesh sponge is preferably prepared from extruded tubular netting mesh which has been prepared from special strong and flexible polymeric material. Extruded tubular netting mesh of this type, and particularly those prepared from polyethylene, have been used for the covering of meat and poultry and are readily available in industry.

The polymeric mesh sponge comprises a plurality of plies of an extruded tubular netting mesh prepared from a strong flexible polymer, preferably of the group consisting of addition polymers of olefin monomers, and polyamides of polycarboxylic acids and polyamines, said plies of tubular netting mesh are folded upon itself numerous times to form a soft ball-like polymeric mesh sponge.

The tubes or stripes of netted mesh polymer can be securely attached by means of a nylon band or suitable closure. This type of polymeric mesh sponge is disclosed in U.S. Pat. No. 4,462,135, Jul. 31, 1984, to Sanford, incorporated herein by reference.

An example of a hand-held ball-like polymeric mesh sponge is disclosed in U.S. Pat. No. 5,144,744, to Campagnali, Sep. 8, 1992, incorporated herein by reference. It is a diamond-mesh polyethylene sponge obtained from a number of netting tubes stretched over supports, joined and bound together at the center and then released from the supports.

Commercially available "polymeric mesh sponges" are sold by The Body Shop and Bynum Concepts, Inc. Other suppliers include Supremia Use in New Jersey, Sponge Factory Dominicana in the Dominican Republic and Integrated Marketing Group in Harrison, N.Y.

The following are some, although certainly not all, specifications for suitable bath polyethylene polymeric mesh sponges:

| Size Dia. | Tubes | Ea. Length | Total Length | Wt. gm. |
|-----------|-------|------------|--------------|---------|
| 3"        | 2     | 60 cm      | 120 cm       | 15      |
| 4"        | 4     | 50 cm      | 200 cm       | 23      |
| 5"        | 4     | 80 cm      | 320 cm       | 37      |

One (1") inch=2.54 cm; 3"=3×2.54 cm; 4"=4×2.54 cm; etc.

FIG. 1 is a perspective representation of a diamond-mesh polymeric hand held ball-like bath sponge showing a rope handle 7 which can be used in the present invention. The ease with which a cleansing polymeric mesh sponge can be held in the hand for cleaning is shown in FIG. 2. A security band 13 hold the multi-layered netting mesh together to form the polymeric mesh sponge. The netting mesh that can be used in making the polymeric mesh sponge is illustrated in FIG. 3, wherein 21 represents the mesh in stretched position. The fine polymeric filaments used in making the netting are represented by 18 with 19 representing the spot bonding of the filaments to form the open mesh 20.

Two 2 netting tubes at 60 cm length each can be used to make a 3-inch ball sponge. They can be bundled manually with a loop or rope to form a ball-like polymeric mesh sponge. Other designs such as rectangular gloves and washing implements made with the mesh material also work very well in the system of the present invention.

FIG. 4 shows a specific type of pouf which may be used. In this pouf there is an opening into which bars may be inserted. Typically there is some form of closure mechanism, e.g., a drawstring around the outside of the bag which can be drawn or closed once the bar is inside. Other closure systems may also be used in theory.

The following examples are intended to better illustrate the invention and are not intended to be limiting in any way.

### EXAMPLES

Bars having the following general formulation were used to determine differences in lather performance.

| % BY WT.                    |            |
|-----------------------------|------------|
| <u>BAR A</u>                |            |
| Fatty acid isethionate      | 40-60%     |
| Free fatty acids            | 15-35%     |
| Sodium isethionate          | 3-8%       |
| Sulfosuccinate              | 3-8%       |
| Betaine                     | 1-5%       |
| Water & minors              | to balance |
| <u>BAR B</u>                |            |
| Fatty acid isethionate      | 25-55%     |
| Polyalkylene glycol         | 20-30%     |
| Free fatty acid             | 5-10%      |
| Betaine                     | 3-8%       |
| Emollient oil               | 2-15%      |
| Starch (e.g., maltodextrin) | 5-10%      |
| Water & minors              | to balance |

Bar B compositions were used with and without a pouf implement.

### Protocol

A consumer study was conducted wherein consumers were given either Bar A, Bar B with pouf or Bar B without pouf to use at home for a period of two weeks and asked to fill out a questionnaire.

Relevant to the subject invention, the following questions relating to lather attributes were presented.

1. The bar provided sufficient lather during the shower;
2. The bar provided sufficient lather during facial washing;

3. The bar lather was bubbly; and
4. The bar lather was thick and creamy.

For each statement, the subjects were giving a choice of 7 responses ranging as follows:

- (1) Disagree completely;
- (2) Disagree strongly;
- (3) Disagree somewhat;
- (4) Neither agree nor disagree;
- (5) Agree somewhat;
- (6) Agree strongly; and
- (7) Agree completely.

Using standard and well known statistical analysis techniques, significant differences were found between the responses for Bar B with pouf compared to Bar B without pouf for statements 1 and 3 above (lather during shower and bubbling). Significant difference is measured at 99.557 and 99.98% confidence levels respectively.

For statement 4 (lather thick and creamy) statistical analysis showed significant difference between Bar B with pouf relative to Bar B without pouf at 94.06 confidence level.

No statistic difference was found of statement 2 relating to facial washing. While not wishing to be bound by theory, this may be because people removed the bars from pouf for facial washing or that differences are not as readily noted when washing the face.

What is claimed is:

1. A cleansing system comprising:

- (1) a cleansing bar composition comprising:
  - (a) 5 to 90% by wt. synthetic surfactant selected from the group consisting of anionic surfactants, nonionic surfactants, amphoteric surfactants, cationic surfactants and mixtures thereof, wherein said surfactant composition comprises at least 15% to 80% by wt. total bar C8 to C24 acyl isethionate;
  - (b) 10% to 90% by wt. of a bar structurant or filler selected from the group consisting of fatty acids and esters or salts thereof; C<sub>8</sub>-C<sub>24</sub> alcohols and ethers thereof; polyalkylene glycols of MW2000 to 100,000; starches and hydrophobically modified water soluble polymer;
  - (c) 1% to 10% by wt. water;
  - (d) about 2 to 15% by wt. emollient oil selected from the group consisting of silicone oils and gums; fats and oils; waxes; hydrophobic plant extracts; hydrocarbons selected from the group consisting of liquid paraffins, vaseline, microcrystalline wax, ceresin, squalene, pristan and mineral oil; essential oils; lipids; vitamins; sunscreens; phospholipids; and mixtures thereof; and
- (2) a light weight polymeric meshed personal cleansing hand held sponge; where said sponge is in a form suitable for use in a hand held cleansing implement and wherein said sponge holds said cleansing bar inserted therein.

2. A composition according to claim 1 comprising 5% to 60% by wt. surfactant.

3. A composition according to claim 1 comprising:

- (a) 5% to 60% by wt. surfactant;
- (b) 10% to 70% by wt. structurant/filler; and
- (c) 2% to 15% by wt. emollient oil.

4. A composition according to claim 1, wherein (a) comprises 10% to 60% by wt. surfactant.

**11**

5. A composition according to claim 1, wherein (b) comprises 20% to 60% by wt. structurant and/or filler.

6. A composition according to claim 4, comprising:

(a) 10% to 60% by wt. surfactant;

**12**

(b) 10% to 35% by wt. structurant/filler; and  
(c) 2% to 10% by wt. emollient.

\* \* \* \* \*